# EUROPEAN PATENT SPECIFICATION

(11) **EP 3 790 950 B1**
(45) Date of publication and mention of the grant of the patent: **01.11.2023**
(21) Application number: 18917802.3
(22) Date of filing: 10.05.2018
(51) Int. Cl.: C11D 1/12, C11D 3/08, C11D 3/10, C11D 1/14, C11D 1/22, C11D 3/04, C11D 9/00, C11D 11/00, C11D 17/06

(54) **DETERGENT GRANULE**
WASCHMITTELGRANULAT
GRANULÉ DÉTERGENT

(43) Date of publication of application: 17.03.2021
(73) Proprietor: The Procter & Gamble Company, Cincinnati, OH 45202 (US)
(72) Inventor: XU, Dan, Beijing 101312 (CN); SHEN, Rui, Beijing 101312 (CN); TIAN, Xiao, Beijing 101312 (CN); GUAN, Zhe, Beijing 101312 (CN); HUANG, Xu, Beijing 101312 (CN)
(74) Representative: P&G Patent Belgium UK
(86) International application number: PCT/CN2018/086291
(87) International publication number: WO 2019/213890

(56) References cited:
- WO-A1-93/18123
- WO-A1-2013/054624
- WO-A1-2013/054624
- WO-A1-2014/198128
- WO-A1-2016/015326
- WO-A1-2018/014281
- WO-A2-2009/050026
- US-A- 6 015 784
- US-A- 6 015 784
- US-A1- 2004 058 843
- US-A1- 2004 058 843

## Description

### FIELD OF THE INVENTION

The present invention relates to a detergent granule that can be used to make cleaning products, especially granular detergent products.

### BACKGROUND OF THE INVENTION

Mid-cut alkyl sulfate (MCAS or AS) with a C₆-C₁₆ branched or unbranched unalkoxylated alkyl group has been discovered effective for suds-boosting when it is used as a co-surfactant with linear alkylbenzene sulphonate (LAS) in cleaning compositions, particularly laundry detergent compositions. For example, WO2009010911 discloses the use of MCAS for boosting suds in a LAS-based surfactant system and forming a detergent composition with a reduced total surfactant level, but without apparently deteriorating the sudsing profile of the detergent composition.

Some MCAS raw materials are available in elongated needle form, which are formed by an extrusion process. This extruded needle form of MCAS material is easy to process, with little or no risk of caking, clumping or clogging up the processing lines. However, the extruded MCAS needles have limited suds-boosting effect when used in combination with LAS in cleaning compositions, probably due to its relatively large size and corresponding poor dissolution profile.

The MCAS raw materials are available in fine powder form with a medium particle size ranging from 200 µm to 1000 µm, which has exhibited good suds-boosting effect when used as a co-surfactant for LAS. However, such fine MCAS powder is prone to caking to clumping at a temperature higher than 35-37°C due to MCAS surfactant phase change as well as its tendency to absorb ambient water when placed in humid environment, and may cause significant processing challenges during shipping and manufacturing.

There is therefore a need to provide MCAS particles with physical characteristics and chemical compositions that can strike an improved balance between good dissolution profile and satisfactory suds-boosting effect on one hand, and reduced risk of caking and clumping and easy of processing/handling on the other hand.

US 6 015 784 A relates to secondary (2,3) alkyl sulfate surfactants that are mixed with organic material such as polyacrylate and compacted to form chips that are subsequently comminuted and then coated with a free-flow aid to form particles that are useful in laundry detergents.

### SUMMARY OF THE INVENTION

The present invention has discovered, surprisingly and unexpectedly, that by making a detergent granule of a relatively small particle size and a relatively low aspect ratio (i.e., its shape is closer to sphere rather than needle), the dissolution profile of such detergent granule can be improved, and the suds-boosting effect is enhanced correspondingly. Further, when such detergent granule contains MCAS at a very high level (e.g., from about 85% to about 95% by weight) in combination with a sufficient amount (e.g., from about 4% to about 14% by weight) of a water-soluble salt, it is less likely to absorb ambient water and therefore less like to cake or form clumps during shipping or storage.

In one aspect, the present invention relates to detergent granule comprising:
a) from about 85% to about 95%, by weight of the detergent granule, of an alkyl sulfate (AS) having a branched or linear unalkoxylated alkyl group comprising from about 6 to about 16 carbon atoms;
b) from about 4% to about 14%, by weight of the detergent granule, of a water-soluble salt selected from the group consisting of sodium sulfate, sodium carbonate, magnesium chloride, magnesium sulfate, sodium silicate, and combinations thereof; and
c) from about 1% to about 5%, by weight of the detergent granule, of water, while the detergent granule is characterized by a Medium Particle Size ranging from about 200 µm to about 1000 µm and an aspect ratio of no more than about 2.

In another aspect, the present invention relates to a cleaning composition comprising from about 0.1% to about 10%, by weight of such cleaning composition, of the above-mentioned detergent granule.

In yet another aspect, the present invention relates to the use of the above-mentioned cleaning composition for hand-washing fabrics.

These and other aspects of the present invention will become more apparent upon reading the following detailed description of the invention.

### BRIEF DESCRIPTION OF THE DRAWINGS

FIG. 1 is a graph showing the dynamic vapor absorption data of an inventive detergent granule according to an embodiment of the present invention, in comparison with that of a comparative detergent granule outside of the scope of the present invention.

### DETAILED DESCRIPTION OF THE INVENTION

Features and benefits of the various embodiments of the present invention will become apparent from the following description, which includes examples of specific embodiments intended to give a broad representation of the invention. Various modifications will be apparent to those skilled in the art from this description and from practice of the invention. The scope of the present invention is not intended to be limited to the particular forms disclosed and the invention covers all modifications, equivalents, and alternatives falling within the scope of the invention as defined by the claims.

As used herein, articles such as "a" and "an" when used in a claim, are understood to mean one or more of what is claimed or described. The terms "comprise," "comprises," "comprising," "contain," "contains," "containing," "include," "includes" and "including" are all meant to be nonlimiting.

As used herein, the term "detergent granule" refers to particles containing one or more detersive actives, including but not limited to surfactants, bleaching agents, enzymes, polymers, chelants, and combinations the"reof.

As used herein, the term "cleaning composition" includes, unless otherwise indicated, granular or powder-form all-purpose or "heavy-duty" washing agents, especially cleaning detergents, for fabrics, as well as cleaning auxiliaries such as bleach, rinse aids, additives, or pre-treat types; hand dishwashing agents or light duty dishwashing agents, especially those of the high-foaming type; machine dishwashing agents; mouthwashes, denture cleaners, car or carpet shampoos, bathroom cleaners; hair shampoos and hair-rinses; shower gels and foam baths and metal cleaners; as well as cleaning auxiliaries such as bleach additives or pre-treat types. In one preferred aspect, the cleaning composition is a solid laundry detergent composition, and more preferably a free-flowing particulate laundry detergent composition (i.e., a granular laundry detergent product).

As used herein, the term "Median Particle Size" refers to the mid-point of the distribution of the particle sizes of the detergent granule, as measured by the Sieve Test as disclosed herein.

As used herein, the term "aspect ratio" refers to the ratio of the largest diameter of an article over the smallest diameter of such article orthogonal to the largest diameter.

As used herein, the term "water-soluble" refers to a solubility of more than about 30 grams per liter (g/L) of deionized water measured at 20°C and under the atmospheric pressure.

As used herein, the terms "consisting essentially of" means that the composition contains less than about 1%, preferably less than about 0.5%, of ingredients other than those listed.

Further, the terms "essentially free of," "substantially free of" or "substantially free from" means that the indicated material is present in the amount of from 0 wt% to about 0.5 wt%, or preferably from 0 wt% to about 0.1 wt%, or more preferably from 0 wt% to about 0.01 wt%, and most preferably it is not present at analytically detectable levels. The term "substantially pure" or "essentially pure" means that the indicated material is present in the amount of from about 99.5 wt% to about 100 wt%, preferably from about 99.9 wt% to about 100 wt%, and more preferably from 99.99 wt% to about 100 wt%, and most preferably all other materials are present only as impurities below analytically detectable levels.

### MCAS

The AS surfactant used in the detergent granule of the present invention contains a branched or linear unalkoxylated alkyl group containing from about 6 to about 16 carbon atoms, and is therefore also referred to as Mid-Cut AS or MCAS.

Preferably, the AS has the generic formula of R-O-SO₃⁻ M⁺, while R is branched or linear unalkoxylated C₆-C₁₆ alkyl group, and M is a cation of alkali metal, alkaline earth metal or ammonium. More preferably, the R group of the AS surfactant contains from about 8 to about 14 carbon atoms, more preferably from about 10 to about 14 carbon atoms, most preferably from about 12 to about 14 carbon atoms. R can be substituted or unsubstituted, and is preferably unsubstituted. R is substantially free of any alkoxylation. M is preferably a cationic of sodium, potassium, or magnesium, and more preferably M is a sodium cation.

Preferably, but not necessarily, the detergent granule of the present invention contains a mixture of C₆-C₁₆ AS surfactants, in which C₈-C₁₄ AS surfactants are present in an amount ranging from about 85% to about 100% by total weight of the mixture. This mixture can be referred to as a "C₈-C₁₄-rich AS mixture." More preferably, such C₈-C₁₄-rich AS mixture contains from about 90 wt% to about 100 wt%, or from 92 wt% to about 98 wt%, or from about 94 wt% to about 96 wt%, or 100 wt% (i.e., pure), of C₈-C₁₄ AS.

In a particularly preferred embodiment of the present invention, the detergent granule contains a mixture of C₆-C₁₆ AS surfactants with from about 30 wt% to about 100 wt% or from about 50 wt% to about 99 wt%, preferably from about 60 wt% to about 95 wt%, more preferably from about 65 wt% to about 90 wt%, and most preferably from about 70 wt% to about 80 wt% of C₁₂ AS. Further, such mixture of C₆-C₁₆ AS surfactants may contain from about 10 wt% to about 100 wt%, preferably from 15 wt% to about 50 wt%, and more preferably from 20 wt% to about 30 wt% of C₁₄ AS. This mixture can be referred to as a "C₁₂-C₁₄-rich AS mixture."

In a most preferred embodiment of the present invention, the detergent granule contains a mixture of AS surfactants that consists essentially of C₁₂ and/or C₁₄ AS surfactants. For example, such mixture of AS surfactant may consist essentially of from about 70 wt% to about 80 wt% of C₁₂ AS and from 20 wt% to about 30 wt% of C₁₄ AS, with little or no other AS surfactants therein. Such mixture may also consist of substantially pure C₁₂ AS, or alternatively, substantially pure C₁₄ AS.

A commercially available AS mixture particularly suitable for practice of the present invention is Texapon^{®} V95 G from Cognis (Monheim, Germany).

Further, the detergent granule of the present invention may contain a mixture of C₆-C₁₆ AS surfactants comprising more than about 50 wt%, preferably more than about 60 wt%, more preferably more than 70 wt% or 80 wt%, and most preferably more than 90 wt% or even at 100 wt% (i.e., substantially pure), of linear AS surfactants having an even number of carbon atoms, including, for example, C₆, C₈, C₁₀, C₁₂, C₁₄, and C₁₆ AS surfactants.

The mixture of C₆-C₁₆ AS surfactants as described can be readily obtained by sulphonation of alcohol(s) with the corresponding numbers of carbon atoms. The required carbon chain length distribution can be obtained by using alcohols with the corresponding chain length distribution prepared either synthetically or extracted/purified from natural raw materials or formed by mixing corresponding pure starting materials. For example, the mixture of C₆-C₁₆ AS surfactants may be derived from naturally occurring triglycerides, such as those contained in palm kernel oil or coconut oil, by chemically processing such triglycerides to form a mixture of long chain alcohols and then sulphonating such alcohols to form AS surfactants. The mixture of alcohols derived from the naturally occurring triglycerides typically contain more than about 20 wt% of C₁₆-C₁₆ alcohols. A mixture containing a lower proportion of C₁₆-C₁₆ alcohols may be separated from the original mixture before the sulphonation step, in order to form the desired mixture of C₆-C₁₆ AS surfactants as described hereinabove. Alternatively, the desired mixture of C₆-C₁₆ AS surfactants can be readily obtained by separating and purifying the already formed AS mixtures. Suitable separation and purification methods include, but are not limited to: distillation, centrifugation, recrystallization and chromatographic separation.

The amount of AS surfactant(s) present in the detergent granule of the present invention may range from about 85 wt% to about 95 wt%, and preferably from about 88 wt% to about 92 wt% by total weight of the composition. With such a high level of AS surfactant(s), the detergent granule of the present invention exhibits a high detersive activity and a very good dissolution profile. In a most preferred embodiment of the present invention, the cleaning composition contains from about 85 wt% to about 95 wt%, preferably from about 88 wt% to about 92 wt%, of an AS mixture consisting essentially of from about 70 wt% to about 80 wt% of C₁₂ AS and from 20 wt% to about 30 wt% of C₁₄ AS.

Detergent granules with higher surfactant levels are typically expected to be more difficult to handle due to their tendency to absorb more water. Therefore, it is a surprising and unexpected discovery of the present invention that the detergent granule of the present invention, while containing such a high level of AS surfactant(s), actually absorbs less water across different relative humidity (RH) ranging from 40% to 80%, in comparison with detergent granules containing lower amounts of AS surfactants, e.g., less than about 85 wt%. Correspondingly, the detergent granule of the present invention is less likely to cake or clump and is easier to handle during storage or shipment.

### Water-Soluble Salt

The water-soluble salt used in the detergent granule of the present invention can be selected from the group consisting of sodium sulfate, sodium carbonate, magnesium chloride, magnesium sulfate, sodium silicate, and combinations thereof. Preferably, the water-soluble salt is selected from sodium sulfate, sodium carbonate, or a combination thereof.

The amount of water-soluble salt present in the detergent granule of the present invention may range from about 4 wt% to about 14 wt%, preferably from about 5 wt% to about 12 wt%, and more preferably from about 6 wt% to about 10 wt%. If the detergent granule contains less than about 4 wt% of the water-soluble salt, it exhibits poorer flowability and is therefore more difficult to handle during storage, shipping and manufacturing. If the detergent granule contains more than about 14 wt% of the water-soluble salt, the amount of AS surfactant in such detergent granule likely must be reduced to less than about 85 wt%, which is undesirable for reasons stated hereinabove.

### Water Content

The detergent granule of the present invention may contain from about 1 wt% to about 5 wt% of water, preferably from about 1.5 wt% to about 4 wt%, more preferably from about 2 wt% to about 3 wt%. Too much water in the detergent granule may adversely affect its flowability and handability.

### Other Ingredients

The detergent granule of the present invention may contain one or more other ingredients, such as silica, zeolite, other surfactants, enzymes, bleach actives, chelants, perfumes, dyes, fluorescent materials, and the like.

Preferably, the detergent granule of the present invention consists essentially of the above-mentioned MCAS, water-soluble salt, and water. More preferably, the detergent granule of the present invention is essentially free of other ingredients.

### Size and Shape of Detergent Granule

The detergent granule of the present invention may be characterized by a Medium Particle Size ranging from about 200 µm to about 1000 µm, preferably from about 250 µm to about 600 µm, more preferably from about 300 µm to about 425 µm.

Further, it may be characterized by an aspect ratio of no more than 2, preferably no more than 1.5, more preferably not more than 1.2, most preferably no more than 1.1. The detergent granule of the present invention preferably has a spherical or substantially spherical shape, which functions to further improve its flowability and handability during storage and shipment.

### Cleaning Composition

The detergent granule of the present invention may be used alone for cleaning, but preferably it is combined with other particles to form a cleaning composition, such as a granular laundry detergent product.

In one aspect, the detergent granule is typically added to the cleaning composition at a level of from about 0.1 wt% to about 10 wt%, preferably from about 0.2 wt% to about 8 wt%, more preferably from about 0.5 wt% to about 5 wt%, by weight of the cleaning composition. Preferably, the cleaning composition is a granular detergent composition.

The detergent granule of the present invention may be combined with other particles such as, for example: surfactant particles, such as anionic detersive surfactant particles (especially those containing LAS) including agglomerates and extrudates, non-ionic detersive surfactant particles including agglomerates or extrudates, and cationic detersive surfactant particles including agglomerates and extrudates; enzyme particles; perfume particles including agglomerates or extrudates of perfume microcapsules, and perfume encapsulates such as starch encapsulated perfume accord particles; polymer particles including soil release polymer particles, cellulosic polymer particles; buffer particles including carbonate salt and/or silicate salt particles, preferably a particle comprising carbonate salt and silicate salt such as a sodium carbonate and sodium silicate co-particle, and particles and sodium bicarbonate; other spray-dried particles; fluorescent whitening particles; aesthetic particles such as coloured noodles or needles or lamellae particles; bleaching particles such as percarbonate particles, especially coated percarbonate particles, including carbonate and/or sulfate coated percarbonate, silicate coated percarbonate, borosilicate coated percarbonate, sodium perborate coated percarbonate; bleach catalyst particles, such as transition metal catalyst bleach particles, and imine bleach boosting particles; performed peracid particles; hueing dye particles; and any mixture thereof.

It is preferred that the cleaning composition of the present invention comprises, in addition to the detergent granule described hereinabove, a C₁₀-C₂₀ linear alkylbenzene sulphonate (LAS), and more preferably such cleaning composition further comprises a fatty acid or salt thereof. The MCAS-containing detergent granule of the present invention may interact with such LAS and fatty acid/salt to provide an improved sudsing profile.

It may also be especially preferred for the cleaning composition to comprise low levels, or even be substantially free, of builder. In a preferred embodiment, the cleaning composition comprises no builder.

### Method of Use

The cleaning composition is typically used for cleaning and /or treating a situs *inter alia* a surface or fabric. As used herein, "surface" may include such surfaces such as dishes, glasses, and other cooking surfaces, hard surfaces, hair or skin. Such method includes the steps of contacting an embodiment of the cleaning composition, in neat form or diluted in a wash liquor, with at least a portion of a surface or fabric, then optionally rinsing such surface or fabric. The surface or fabric may be subjected to a washing step prior to the aforementioned rinsing step. For purposes of the present invention, "washing" includes but is not limited to, scrubbing, wiping, and mechanical agitation.

The composition solution pH is chosen to be the most complimentary to a target surface to be cleaned spanning broad range of pH, from about 5 to about 11. For personal care such as skin and hair cleaning pH of such composition preferably has a pH from about 5 to about 8 for laundry cleaning compositions pH of from about 8 to about 10. The compositions are preferably employed at concentrations of from about 200 ppm to about 10,000 ppm in solution. The water temperatures preferably range from about 5 °C to about 100 °C.

In one aspect, a method of laundering fabrics using the cleaning composition of the present invention is disclosed. The method may comprise the steps of contacting a fabric to be laundered with the cleaning composition or a wash liquor formed thereby. The fabric may comprise most any fabric capable of being laundered in normal consumer use conditions.

The cleaning composition herein is especially well-suited for use in a hand-washing context. It can also be used in automatic mashing washing using a top-loading or front-loading automatic washing machine.

The cleaning composition may be employed at concentrations of from about 500 ppm to about 15,000 ppm in solution, and optionally, more dilute wash conditions can be used. Optionally, 50 g or less, or 45 g or less, or 40 g or less, or 35 g or less, or 30 g or less, or 25 g or less, or 20 g or less, or even 15 g or less, or even 10 g or less of the cleaning composition is dissolved into water to form a wash liquor. The wash liquor preferably has a pH of from about 8 to about 10.5. The wash liquor may comprise 40 litres or less of water, or 30 litres or less, or 20 litres or less, or 10 litres or less, or 8 litres or less, or even 6 litres or less of water. The wash liquor may comprise from above 0 to 15 litres, or from 2 litres, and to 12 litres, or even to 8 litres of water. For dilute wash conditions, the wash liquor may comprise 150 litres or less of water, 100 litres or less of water, 60 litres or less of water, or 50 litres or less of water, especially for hand washing conditions, and can depend on the number of rinses. The water to fabric ratio is typically from about 1:1 to about 30:1. Typically, from 0.01 Kg to 2 Kg of fabric per litre of wash liquor is dosed into the wash liquor.

It is preferable that the cleaning composition can be used in hard water conditions where the water hardness is between about 17 ppm to about 600 ppm; or from about 34 ppm to about 340 ppm; or from about 51 ppm to about 300 ppm of hard water ions such as Ca²⁺, Mg⁺, etc., or such as Ca²⁺ and Mg²⁺. It is also preferable that the cleaning composition can be used in cold water temperature, where the temperature is from about 5 °C to about 40 °C, or from about 20 °C to about 30 °C, or from about 15 °C to about 25 °C, as well as all other combinations within the range of about 15 °C to about 35 °C, and all ranges within 10 °C to 40 °C.

### TEST METHODS

The following techniques must be used to determine the properties of the detergent granules and detergent compositions of the invention in order that the invention described and claimed herein may be fully understood.

### TEST 1: Median Particle Size Test Method (Sieve Test Method)

This test method can be used to determine the Median Particle Size of the detergent granules of the present invention. The particle size distribution of the detergent granules is measured by sieving the granules through a succession of sieves with gradually smaller dimensions. The weight of material retained on each sieve is then used to calculate a particle size distribution and Median Particle Size.

This test is conducted to determine the Median Particle Size of the subject particle using ASTM D 502 - 89, "Standard Test Method for Particle Size of Soaps and Other Detergents", approved May 26, 1989, with a further specification for sieve sizes used in the analysis. Following section 7, "Procedure using machine-sieving method," a nest of clean dry sieves containing U.S. Standard (ASTM E 11) sieves #8 (2360 µm), #12 (1700 µm), #16 (1180 µm), #20 (850 µm), #30 (600 µm), #40 (425 µm), #50 (300 µm), #70 (212 µm), and #100 (150 µm) is required. The prescribed Machine-Sieving Method is used with the above sieve nest. The detergent granule of interest is used as the sample. A suitable sieve-shaking machine can be obtained from W.S. Tyler Company of Mentor, Ohio, U.S.A. The data are plotted on a semi-log plot with the micron size opening of each sieve plotted against the logarithmic abscissa and the cumulative mass percent (Q3) plotted against the linear ordinate.

An example of the above data representation is given in ISO 9276-1:1998, "Representation of results of particle size analysis - Part 1: Graphical Representation", Figure A.4. The Median Particle Size (D₅₀) is defined as the abscissa value at the point where the cumulative mass percent is equal to 50 percent, and is calculated by a straight-line interpolation between the data points directly above (a50) and below (b50) the 50% value using the following equation: ${D}_{50} = 10 \left[Log\left({D}_{a 50}\right)-\left(Log\left({D}_{a 50}\right)-Log\left({D}_{b 5 o}\right)\right)∗\left({Q}_{a 5 o}-50%\right)/\left({Q}_{a 50}-{Q}_{bso}\right)\right]$ where Qa₅₀ and Q_{b50} are the cumulative mass percentile values of the data immediately above and below the 50^{th} percentile, respectively; and Dₐ₅₀ and D_{b50} are the micron sieve size values corresponding to these data. In the event that the 50^{th} percentile value falls below the finest sieve size (150 µm) or above the coarsest sieve size (2360 µm), then additional sieves must be added to the nest following a geometric progression of not greater than 1.5, until the median falls between two measured sieve sizes.

### TEST 2: Moisture Content Measurement

Two (2) grams of a sample detergent granule is tested in the Mettler Toledo HR73 Halogen moisture analyzer at 115°C for 40 minutes. The percentage (%) of lost mass at the end of the measurement is recorded as the moisture content of the sample detergent granule.

### EXAMPLES

### Example 1: Comparative Test Showing Reduced Water Absorption by Inventive Detergent Granule

Two sample detergent granules are made, which include an inventive sample of detergent granule containing about 88% MCAS (containing about 65 wt% C12 species, 25 wt% C14 species, 7 wt% C16 species, and no more than 3 wt % other species), 9.5% sodium sulfate, and 2.5% water 90% MCAS and 10% sodium sulfate by total dry weight of such detergent granule (within the scope of the present invention) and a comparative sample of detergent granule containing 78% MCAS (same composition as above), 19.5% sodium sulfate, and 2.5% water by total dry weight of such detergent granule (outside the scope of the present invention).

Each sample detergent granule is formed by adding a specific amount of sodium sulfate into a heated concentrated MCAS paste (containing 74 wt% MCAS in water) and then mixed at an elevated temperature ranging from 60-80°C in a temperature controlled reactor for 10 minutes. The mixture is then manually spread onto a flat surface to form a thin layer having a thickness of about 3-10 mm, which is dried in an oven for about 2 hours at an elevated temperature of 110°C. Once the dried mixture reaches a target moisture content of about 2-3%, it is removed from the oven and ground into a powder form by using a Fritsch Pulverisette 14 grinder (commercially available from Fritsch GmbH, Idar-Oberstein, Germany) at a speed setting of 6 and using a 1.5mm sieve. The powders so formed are further sieved to reach the same particle size distribution as follows:

**TABLE 1**

| Sieve Size (µm) | Mass% of Sample from Each Sieve (g) | Cumulative Mass% Finer (CMPF) |
|---|---|---|
| 850 | 6.33 | 6.33% |
| 600 | 10.33 | 16.69% |
| 425 | 13.23 | 29.93% |
| 250 | 21.81 | 51.74% |
| 150 | 17.88 | 69.62% |
| pan | 30.42 | 100.0% |

The moisture sorption isotherms of both the inventive detergent granule and the comparative detergent granule are acquired using a SPS-11 moisture sorption analyzer (commercially available from ProUmid GmbH & Co. KG, Ulm, Germany). The measurement is started at a relative humidity (RH) of 0% and is gradually increased in steps of about 10% RH each to a final RH of about 80%. The equilibrium condition for each step is set to a mass constancy of ±0.01% over 30 minutes. Temperature of the test condition is set at 35±0.1°C. The delta mass (dm) in % at each RH%, which is an indicator of the percentage of water absorbed by the sample detergent granule at the respective RH%, is calculated by the equation below: $dm in % = \frac{Mass after vapor sorption}{Mass at 0 % RH} \times 100 %$

FIG. 1 is a dynamic vapor absorption graph plotting the delta mass (dm in %) of the inventive detergent granule as well as that of the comparative detergent granule across a RH range RH of from about 40% to about 80%. It is evident that the inventive detergent granule absorbs less water than the comparative detergent granule across at relatively high humidity conditions (e.g., with RH ranging from about 40% to about 80%). Therefore, the inventive detergent granule is less likely to cake or clump when stored or shipped in countries or regions where humidity may present a challenge.

### Example 2: Comparative Test Showing Reduced Caking of Inventive Detergent Granules in Big Bag Test

Five (5) sample detergent granules with the following compositional makeups are made, which include four (4) inventive samples of detergent granules A-E within the scope of the present invention and one (1) comparative sample of detergent granule C1 outside the scope of the present invention:

**TABLE 2**

| **Ingredients (wt%)** | **C1** | **A** | **B** | **D** | **E** |
|---|---|---|---|---|---|
| MCAS | 97.5 | 88 | 88 | 88 | 88 |
| Sodium Carbonate | - | 9.5 | - | - | - |
| Sodium Sulfate | - | - | 9.5 | - | - |
| Magnesium Chloride | - | - | - | 9.5 | - |
| Sodium Silicate | - | - | - | - | 9.5 |
| Water | 2.5 | 2.5 | 2.5 | 2.5 | 2.5 |

Each sample detergent granule is formed by the same method described in Example 1.

Big bag test is used to probe and qualitatively evaluate potential issues with a material prior to shipping such material in a big bag, during which it may be exposed to elevated temperatures. During a big bag test, 100g+/-1g of a test material is first place into a plastic beaker and ensure that the top surface of the test material is level. A second beaker is placed into the first beaker containing the test material, while the bottom of the top, second beaker rests upon the test material, without pushing or forcing the top, second beaker into the test material. The two beakers are sealed together with a PVC tape. A 3Kg mass is placed into the top, second beaker so that the top, second beaker acts as a load-bearing surface for the 3Kg mass upon the test material. The beakers with the test material and the 3Kg mass are then placed in an oven at 35°C and 80%RH. After 20 hours under such test conditions, the 3kg mass is removed, and the test material is cooled down to ambient temperature (with a minimum cooling time of 1 hour). The bottom, first beaker containing the cooled test material is inverted to observe how easy/difficult the test material can flow out of the bottom, first beaker. The flowability of the test material is graded using the following grading scales:

| | |
|---|---|
| • 10: | Free flowing. |
| • 9½: | Slight hesitation, not quite free flowing, but not caked |
| • 9: | Caked, but breaks up on inversion to give a powder. |
| • 8½: | Caked, but breaks up on re-tilting several times. |
| • 8: | Caked, but breaks up with gentle shaking. |
| • 7: | Caked, but breaks up with moderate shaking. |
| • 6: | Caked, but breaks up with vigorous shaking |
| • 5: | Caked, but breaks up with violent shaking. |
| • 4: | Caked solid |

Following are the big bag test results of the five (5) samples of detergent granules:

**TABLE 4**

| | **C1** | **A** | **B** | **D** | **E** |
|---|---|---|---|---|---|
| **Big Bag Grading Score** | 7 | 9.5 | 9.5 | 9.5 | 9.5 |

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm."

The citation of any document is not an admission that it is prior art with respect to any invention disclosed or claimed herein or that it alone, or in any combination with any other reference or references, teaches, suggests or discloses any such invention. Further, to the extent that any meaning or definition of a term in this document conflicts with any meaning or definition of the same term in a document cited herein, the meaning or definition assigned to that term in this document shall govern.

While particular embodiments of the present invention have been illustrated and described, it would be obvious to those skilled in the art that various other changes and modifications can be made without departing from the scope of the invention, as defined by the claims. It is therefore intended to cover in the appended claims all such changes and modifications that are within the scope of this invention.

## Claims

1. A detergent granule comprising:
a) from 85% to 95%, by weight of said detergent granule, of an alkyl sulfate (AS) having a branched or linear unalkoxylated alkyl group comprising from 6 to 16 carbon atoms;
b) from 4% to 14%, by weight of said detergent granule, of a water-soluble salt selected from the group consisting of sodium sulfate, sodium carbonate, magnesium chloride, magnesium sulfate, sodium silicate, and combinations thereof; and
c) from 1% to 5%, by weight of said detergent granule, of water,
wherein said detergent granule is **characterized by** a Medium Particle Size ranging from 200 µm to 1000 µm and an aspect ratio of no more than 2, as determined by the sieve test method described in the description.

2. The detergent granule of claim 1, wherein the branched or linear unalkoxylated alkyl group of said AS comprises from 8 to 14, preferably from 10 to 14, more preferably from 12 to 14 carbon atoms.

3. The detergent granule of claim 1 or 2, wherein said water-soluble salt is selected from the group consisting of sodium sulfate, sodium carbonate, and combination thereof.

4. The detergent granule according to any one of the preceding claims, wherein the Medium Particle Size of said detergent granule ranges from 250 µm to 600 µm, preferably from 300 µm to 425 µm.

5. The detergent granule according to any one of the preceding claims, wherein the aspect ratio of said detergent granule is no more than 1.5, preferably no more than 1.2, more preferably no more than 1.1.

6. A cleaning composition comprising from 0.1% to 10%, by weight of said cleaning composition, of the detergent granule according to any one of the preceding claims.

7. The cleaning composition according to claim 6, wherein the detergent granule is present in an amount ranging from 0.2% to 8%, preferably from 0.5% to 5%, by weight of said cleaning composition.

8. The cleaning composition according to claim 6 or 7, further comprising: (1) a C₁₀-C₂₀ linear alkylbenzene sulphonate (LAS); and (2) a fatty acid or salt thereof.

9. The cleaning composition according to claim 8, wherein said LAS is present in an amount ranging from 6% to 15%, preferably from 7% to 13%, by weight of said cleaning composition; and wherein said fatty acid or salt is present in an amount ranging from 2% to 6%, preferably from 2.5% to 4%, by weight of said cleaning composition.

10. Use of the cleaning composition according to any one of claims 6-9 for hand-washing fabrics.

## Patentansprüche

1. Waschmittelgranalie, umfassend:
a) von zu 85 Gew.-% bis 95 Gew.-% der Waschmittelgranalie, ein Alkylsulfat (AS), das eine verzweigte oder lineare unalkoxylierte Alkylgruppe aufweist, umfassend von 6 bis 16 Kohlenstoffatome;
b) von zu 4 Gew.-% bis 14 Gew.-% der Waschmittelgranalie, ein wasserlösliches Salz, das ausgewählt ist aus der Gruppe bestehend aus Natriumsulfat, Natriumcarbonat, Magnesiumchlorid, Magnesiumsulfat, Natriumsilikat und Kombinationen davon; und
c) von zu 1 Gew.-% bis 5 Gew.-% der Waschmittelgranalie, Wasser,
wobei die Waschmittelgranalie **durch** eine mittlere Teilchengröße in einem Bereich von 200 µm bis 1000 µm und ein Seitenverhältnis von nicht mehr als 2, wie durch das in der Beschreibung beschriebene Siebprüfverfahren bestimmt, **gekennzeichnet ist.**

2. Waschmittelgranalie nach Anspruch 1, wobei die verzweigte oder lineare unalkoxylierte Alkylgruppe des AS von 8 bis 14, vorzugsweise von 10 bis 14, mehr bevorzugt von 12 bis 14 Kohlenstoffatome umfasst.

3. Waschmittelgranalie nach Anspruch 1 oder 2 wobei das wasserlösliche Salz ausgewählt ist aus der Gruppe bestehend aus Natriumsulfat, Natriumcarbonat und Kombination davon.

4. Waschmittelgranalie nach einem der vorstehenden Ansprüche, wobei die mittlere Teilchengröße der Waschmittelgranalie in einem Bereich von 250 µm bis 600 µm, vorzugsweise von 300 µm bis 425 µm, liegt.

5. Waschmittelgranalie nach einem der vorstehenden Ansprüche, wobei das Seitenverhältnis der Waschmittelgranalie nicht mehr als 1,5, vorzugsweise nicht mehr als 1,2, mehr bevorzugt nicht mehr als 1,1, beträgt.

6. Reinigungszusammensetzung, umfassend von zu 0,1 Gew.-% bis 10 Gew.-% der Reinigungszusammensetzung, die Waschmittelgranalie nach einem der vorstehenden Ansprüche.

7. Reinigungszusammensetzung nach Anspruch 6, wobei die Waschmittelgranalie in einer Menge gegenwärtig ist, die in einem Bereich von 0,2 Gew.-% bis 8 Gew.-%, vorzugsweise von 0,5 Gew.-% bis 5 Gew.-%, der Reinigungszusammensetzung liegt.

8. Reinigungszusammensetzung nach Anspruch 6 oder 7, ferner umfassend: (1) ein lineares C₁₀-C₂₀-Alkylbenzolsulfonat (LAS); und (2) eine Fettsäure oder ein Salz davon.

9. Reinigungszusammensetzung nach Anspruch 8, wobei das LAS in einer Menge gegenwärtig ist, die in einem Bereich von 6 Gew.-% bis 15 Gew.-%, vorzugsweise von 7 Gew.-% bis 13 Gew.-%, der Reinigungszusammensetzung liegt; und wobei die Fettsäure oder das Salz in einer Menge gegenwärtig ist, die in einem Bereich von 2 Gew.-% bis 6 Gew.-%, vorzugsweise von 2,5 Gew.-% bis 4 Gew.-%, der Reinigungszusammensetzung liegt.

10. Verwenden der Reinigungszusammensetzung nach einem der Ansprüche 6 bis 9 zum Waschen von Stoffen per Hand.

## Revendications

1. Granule de détergent comprenant :
a) de 85 % à 95 %, en poids dudit granule de détergent, d'un sulfate d'alkyle (AS) ayant un groupe alkyle non alcoxylé ramifié ou linéaire comprenant de 6 à 16 atomes de carbone ;
b) de 4 % à 14 %, en poids dudit granule de détergent, d'un sel hydrosoluble choisi dans le groupe constitué par sulfate de sodium, carbonate de sodium, chlorure de magnésium, sulfate de magnésium, silicate de sodium, et combinaisons de ceux-ci ; et
c) de 1 % à 5 %, en poids dudit granule de détergent, d'eau,
ledit granule de détergent étant **caractérisé par** une taille moyenne de particules allant de 200 µm à 1000 µm et un rapport d'aspect n'excédant pas 2, comme déterminé par le procédé de test de tamisage décrit dans la description.

2. Granule de détergent selon la revendication 1, dans lequel le groupe alkyle non alcoxylé ramifié ou linéaire dudit AS comprend de 8 à 14, de préférence de 10 à 14, plus préférablement de 12 à 14 atomes de carbone.

3. Granule de détergent selon la revendication 1 ou 2, dans lequel ledit sel hydrosoluble est choisi dans le groupe constitué par sulfate de sodium, carbonate de sodium, et combinaison de ceux-ci.

4. Granule de détergent selon l'une quelconque des revendications précédentes, dans lequel la taille moyenne de particules dudit granule de détergent va de 250 µm à 600 µm, de préférence de 300 µm à 425 µm.

5. Granule de détergent selon l'une quelconque des revendications précédentes, dans lequel le rapport d'aspect dudit granule de détergent n'est pas supérieur à 1,5, de préférence pas supérieur à 1,2, plus préférablement pas supérieur à 1,1.

6. Composition de nettoyage comprenant de 0,1 % à 10 %, en poids de ladite composition de nettoyage, du granule de détergent selon l'une quelconque des revendications précédentes.

7. Composition de nettoyage selon la revendication 6, dans laquelle le granule de détergent est présent en une quantité allant de 0,2 % à 8 %, de préférence de 0,5 % à 5 %, en poids de ladite composition de nettoyage.

8. Composition de nettoyage selon la revendication 6 ou 7, comprenant en outre : (1) un sulfonate d'alkylbenzène linéaire (LAS) en C₁₀ à C₂₀ ; et (2) un acide gras ou sel de celui-ci.

9. Composition de nettoyage selon la revendication 8, dans laquelle ledit LAS est présent en une quantité allant de 6 % à 15 %, de préférence de 7 % à 13 %, en poids de ladite composition de nettoyage ; et dans laquelle ledit acide gras ou sel est présent en une quantité allant de 2 % à 6 %, de préférence de 2,5 % à 4 %, en poids de ladite composition de nettoyage.

10. Utilisation de la composition de nettoyage selon l'une quelconque des revendications 6 à 9 pour le lavage à la main de tissus.
